

# UNITED STATES PATENT OFFICE.

CLARENCE H. BRYCE, OF GLEN RIDGE, NEW JERSEY, ASSIGNOR TO BENJAMIN MOORE & CO., OF BROOKLYN, NEW YORK, A CORPORATION OF NEW JERSEY.

## SOUND-ABSORBING COATING.

1,341,704.

Specification of Letters Patent.

Patented June 1, 1920.

No Drawing.

Application filed September 18, 1919. Serial No. 324,284.

To all whom it may concern:

Be it known that I, CLARENCE HILL BRYCE, a citizen of the United States, residing at No. 13 Windsor Place, Glen Ridge, in the 5 county of Essex and State of New Jersey, have invented a new and useful composition of matter called sound absorbing coatings to be used as a sound-absorbing coating for acoustic effects on the walls and ceiling 10 of offices, rooms, and halls, of which the following is a specification.

The objects of my improvement are:

First:—To provide means for absorbing noise and objectionable sounds in offices, 15 rooms and halls so that they may the less interfere with discussion and speech going on therein;

Second:—At the same time to provide a coating that can be used on any surface 20 where an oil paint would ordinarily be used, and which may be used as a decorative coating and in conjunction with its noise absorbing effect, has a high coefficient of light reflection;

25 Third:—To provide a coating that is light in weight, elastic and which adheres firmly to the surface and dries with a smooth flat finish and is durable and reasonably cheap;

Fourth:—To render offices, rooms and 30 halls which are invaded with stray noises or other objectionable sounds or which contain within themselves noisy conditions as from the rustling and foot shuffling of an audience, more available and comfortable 35 for speech from the stage or from the discussion of the occupants or otherwise, by the sound absorbing effect of my improved coating on the walls and ceilings, however applied.

40 My improved coating is composed of a liquid vehicle and a light gravity pigment of fine texture; the vehicle being composed of gums, such as rubber, caoutchouc, balata gum, gutta percha and the like, dissolved in benzin, naphtha, turpentine substitutes or 45 any similar volatile solvents, and when this vehicle is mixed with the pigment, it must form an elastic and flexible coating that will adhere to almost any surface. The pigment shall be very fine in texture, light in 50 gravity and have a high coefficient of light reflection.

I will now describe my composition as consisting of the preferred ingredients

combined in the preferable proportions 55 and in the preferred manner as follows, namely:—

125 pounds of carbonate of magnesium, and 100 gallons of vehicle.

The vehicle consists of 11 pounds of light 60 grizzly crape rubber, and 47 gallons of volatile mineral spirits such as texene, varnolene or the like.

The method of making is as follows: The rubber is cut into small pieces and agitated 65 continuously for several days with the volatile mineral spirits until it is completely in solution. The pigment is next mixed with this liquid by agitating in a paint-mixer and then ground through a Burr stone mill. It 70 is then ready for use if required as a white coating or if desired it may be tinted to any shade by the admixture of small amounts of tinting color either dry or ground in oil, depending upon the shade required. If a 75 large amount of color is required, it must be ground in the vehicle as a large addition of linseed or other drying oil will harden the coating and tend to counteract the effect of the same for its sound absorbing qualities.

For the best results felt fabric, which may be as much as an inch thick or may be less is applied to a plastered ceiling or to the ordinary plastered walls fastened thereto by 85 some adhesive substance or otherwise, then narrow battens of wood spaced preferably from 3 to 6 feet apart are applied to the felt surface, over which is stretched a very light weight fabric, nainsook, silk or even paper 90 or any membranous substance leaving an air space between the fabric and the felt of about an inch; to this latter fabric is applied my improved composition of matter 95 in a single thin coat with a brush or by a spray or otherwise as ordinary paint may be applied, but with smaller effect my composition of matter may be applied direct to the plastered wall or direct to the thin fabric applied to the plastered wall or any 100 other way. It may be applied to new constructions or to existing offices and auditoriums preventing objectionable hum and noise and echoes, and I thus realize all the foregoing objects.

I do not restrict myself to the substances, ingredients or processes named but I claim all the known physical and chemical equiva-

lents or any processes that will produce an available coating and absorb sound whether the composition also reflects light or not.

Other paints have a tendency to shrink the fabric, draw it tight and harden it producing a drum-head effect, reflecting sound and accenting the objections that I remove. With some other paints the pores of the fabric are not sufficiently filled and dust 10 works up into the air space and afterward works back through the fabric and hangs down in strings somewhat as it does through an unpainted fabric, disfiguring the ceiling and shaking down on any concussion on 15 the floor above. My coating fills the interstices in the fabric without lessening the sound absorbing effect. It thus has sanitary values.

Instead of carbonate of magnesia, I have 20 used diatomaceous earth with good effect and I may use with some effect any pigment of light gravity that fills the interstices of the fabric, without excess hardening or drum-head effect, and therefore I claim such 25 physical equivalent.

I am not aware that all the ingredients of my composition have been used together for any purpose but as an article of manu-

facture, as well as a composition of matter for its acoustic values in absorbing objectionable sound and noise, I regard my discovery as absolutely new.

What I claim and desire to secure by Letters Patent is:

1. The herein described composition of matter and article of manufacture consisting of carbonate of magnesium and a vehicle consisting of rubber and volatile spirits substantially as described and for the purpose specified. 35 40

2. The herein described composition of matter and article of manufacture for deadening sound, consisting of 125 pounds of carbonate of magnesium and 100 gallons of vehicle which consists of volatile mineral spirits and rubber in substantially the proportions of forty seven gallons of the spirits to eleven pounds of the rubber. 45

In witness whereof, I have hereunto set my hand at this city, county and State of 50 New York, this 9th day of September, 1919.

CLARENCE H. BRYCE.

In presence of—

HOWARD O. PIERSON,  
RUDOLPH C. BURGMANN.